

## UNITED STATES PATENT OFFICE

2,175,806

## PROCESS OF PRODUCING WATER-INSOLUBLE AZO DYESTUFFS ON THE FIBER AND DYEING PREPARATIONS THEREFOR

Karl Jellinek, Offenbach-on-the-Main, Germany,  
assignor to General Aniline Works, Inc., New  
York, N. Y., a corporation of Delaware

No Drawing. Application April 21, 1938, Serial  
No. 203,445. In Germany April 23, 1937

11 Claims. (Cl. 8—46)

The present invention relates to a process of producing water-insoluble azo dyestuffs on the fiber and to dyeing preparations therefor.

In the production of azo dyestuffs on the fiber there are added to the developing baths buffering substances capable of preventing damage of the diazo solution by the alkali of the grounding solution. As alkali binding agents of this kind aluminium sulfate, zinc sulfate and magnesium sulfate are preferred. The salt is advantageously mixed with the commercial dye-salt so that the dyer has at his disposal a diazo preparation which, by simple dissolution in water, yields a developing bath ready for dyeing and requiring no further addition, as is necessary if, for instance, acetic acid is used as alkali binding agent.

The use of these buffering substances, however, involves certain disadvantages insofar as they are liable to form with the textile oils present in the grounding solution—generally Turkey red oil—metal soaps which are, for the most part, of a smeary consistency and can deposit on the fiber; this may spoil the spinning capacity of loose material and may lead to wetting defects of piece goods, whereby the dyeings obtained are non-uniform.

I have found that such disadvantages are avoided by conducting the coupling operation in the presence of a water-soluble chromic salt. As such salts there may be used, for instance, chromic sulfate, chromic fluoride or chromic acetate. The chromic salts are very suitable as alkali binding agents. When used with diazo compounds of feeble coupling power they do not give rise to insufficient yields of dyestuff, as is often the case when aluminium sulfate or zinc sulfate is used, and have the advantage over magnesium sulfate that they have a feebly acid reaction and thus influence favorably the clarity of the dyeings. Furthermore, there are not formed injurious deposits on the fiber so that a better and more uniform appearance of the goods is guaranteed.

Which of the chromic salts in question is most suitable for attaining an optimum dyeing with the selected base can be ascertained in an easy manner by a preliminary test.

It is also possible previously to mix water-soluble chromic salts with diazonium-compounds, which have separated in solid form, from bases

suitable for the preparation of ice-colors, or with bases of this kind in admixture with the quantity of nitrite as is necessary for the diazotization, or with such bases or their mineral acid salts. In the first case dyeing preparations are obtained which yield by simple dissolution in water dye-baths ready for use, whereas the dyeing preparations furthermore mentioned allow to prepare developing baths by introduction into mineral acids or by simple diazotization. The dyeing preparations thus obtained are distinguished by their stability, even when they contain besides the solid diazonium compound chromic acetate which in many cases is especially suitable as a buffering agent. This could not be foreseen, since with other metal salts of organic acids, as, for instance, aluminium acetate, experiments have shown that stable diazo preparations cannot be obtained. The dyeing preparations may furthermore contain the usual adjuvants or diluents.

The following examples serve to illustrate the invention, but they are not intended to limit it thereto:

1. 29.75 grams of zinc chloride double salt of diazotized 2-amino-6-benzoylamino-4-methoxy-1-methylbenzene in the form of a press cake of 80 per cent. strength are triturated to a homogeneous powder together with 20 grams of anhydrous sodium sulfate and 50 grams of chromic acetate.

A dyeing preparation is obtained which by simple dissolution in water yields developing solutions ready for use.

Instead of chromic acetate the same quantity of chromic fluoride may be used.

2. 49.63 grams of the zinc chloride double salt of diazotized 1-amino-4-benzoylamino-2,5-diethoxybenzene in the form of a moist press cake are dehydrated under reduced pressure and finely triturated in admixture with 40 grams of chromic formate and 10 grams of sodium sulfate.

A dyeing preparation is obtained which by sim-

ple dissolution in water yields developing solutions ready for use.

3. 30 grams of the diazonium chloride from 4-amino-4'-methoxydiphenylamine dried under reduced pressure are finely triturated together with 65 grams of chromic acetate.

A dyeing preparation is obtained which by simple dissolution in water yields developing solutions ready for use.

4. 26 grams of the diazonium chloride from 4-amino-diphenylamine dried under reduced pressure are finely triturated with

15 65 grams of chromic oxalate and 10 grams of anhydrous sodium sulfate.

A dyeing preparation is obtained which by simple dissolution in water yields a developing solution ready for use.

20 5. 40 grams of the zinc chloride double salt of tetrazotized dianisidine are dried under reduced pressure, mixed with

20 grams of anhydrous sodium sulfate and

25 40 grams of chromic fluoride and triturated.

A dyeing preparation is obtained which by simple dissolution in water yields a developing solution ready for use.

30 6. 18.2 grams of the hydrochloride of 1-amino-3-chlorobenzene of 90 per cent. strength are triturated together with 23.8 grams of hydrous chromic sulfate. A stable preparation is obtained which when diazotized in the usual manner and neutralized yields dye baths ready for use.

35 7. 30 grams of the hydrochloride of 85 per cent. strength of 4-chloro-2-aminodiphenyl ether are mixed with 12 grams of hydrous chromic fluoride. A stable preparation is obtained which when diazotized in the usual manner and neutralized yields dye baths ready for use.

40 8. 28.5 grams of the hydrochloride of 1-amino-2-methoxy benzene-5-sulfonic acid-diethylamide of 90 per cent. strength are triturated together with 33 grams of hydrous chrome alum. A stable preparation is obtained which when diazotized in the usual manner and neutralized yields dye-baths ready for use.

In the same manner the corresponding quantity of metaaminoazotoluene or 2,4-dibromo-1-aminonaphthalene may be mixed with the quantity of hydrous chrome alum indicated above. Also in this case a stable preparation is obtained which when diazotized in the usual manner and neutralized yields dye-baths ready for use.

55 9. 16.8 grams of 5-nitro-2-amino-1-methoxybenzene are mixed with 8 grams of sodium nitrite and 12 grams of hydrous chromic fluoride. A stable preparation is obtained which may be diazotized by introduction into dilute hydrochloric acid and which yields after neutralization by means of sodium acetate developing solutions ready for use in dyeing.

60 10. 31.1 grams of the zinc chloride double salt of diazotized 1-aminoanthraquinone are mixed in the form of a moist press cake together with 10 grams of anhydrous sodium sulfate and 60 grams of hydrous chromic acetate. After drying a stable dyeing preparation is obtained which by dissolution in water yields dye-baths ready for use.

65 11. Cotton yarn is impregnated in the vat at 30° C. in a solution containing per liter

2.3-hydroxynaphthoylaminobenzene--grams 6

Caustic soda solution of 34° Bé-----cc 9

Formaldehyde of 33 per cent. strength-----cc 6

75 Turkey red oil-----cc 10

for 30 minutes, the proportion of the goods to the liquor being 1:20; the yarn is squeezed and developed in the vat for 20 minutes, the proportion of the goods to the liquor being 1:20, in a diazo-solution which has been neutralized with sodium acetate and contains the amount of diazo-compound corresponding with 3.5 grams of 1-amino-2-nitro-4-chlorobenzene per liter, and to which 0.8 gram of chromic chloride per liter has been added. After thoroughly rinsing, while cold, and, if necessary, acidifying, the dyeing is after-treated at boiling temperature for 30 minutes with a solution containing 3 grams of soap and 1 gram of calcined sodium carbonate per liter. A yellowish red tint is thus obtained.

10 12. Cotton yarn is impregnated in a solution prepared as described in Example 11 and containing per liter 7 grams of 1-(2',3'-hydroxynaphthoylaminoo)-2-methylbenzene, the dyeing is then developed in a diazo-solution prepared in the usual manner, neutralized with sodium acetate and containing the amount of diazo-compound corresponding with 1.3 grams of 1-amino-3-chlorobenzene per liter and 0.55 gram of chromic fluoride, and is after-treated in the usual manner.

15 A reddish orange tint is obtained.

Instead of the diazo-solution prepared from the base there may be used the solution of a dye preparation which contains 0.55 gram of chromic fluoride for the quantity of diazonium compound corresponding with 1.8 grams of 1-amino-3-chlorobenzene in the form of the acid 1,5-naphthalene-disulfonate, and one of the usual adjuvants.

20 13. Cotton yarn is impregnated in the usual manner in a solution containing per liter—

1-(2',3'-hydroxynaphthoylaminoo)-2-methoxybenzene-----grams 5  
Caustic soda solution of 34° Bé-----cc 7.5 40  
Formaldehyde of 33 per cent. strength-----cc 5  
Turkey red oil-----cc 10

squeezed and developed in a diazo-solution, neutralized by means of sodium acetate which contains the quantity of diazo-compound corresponding with 1.4 grams of 1-amino-2-methyl-5-chlorobenzene and 1.4 grams of hydrous chromic sulfate per liter, and after-treated in the usual manner.

25 A clear scarlet tint is obtained.

Instead of the diazo-solution prepared from the base there may be used the solution of a diazo-salt preparation containing for the quantity of diazo-compound corresponding with 1.4 grams of 1-amino-2-methyl-5-chlorobenzene in the form of the acid 1,5-naphthalene-disulfonate, 1.4 grams of hydrous chromic sulfate and one of the usual adjuvants.

30 14. 80 grams of 1-amino-2-methyl-4-chlorobenzene hydrochloride of 90 per cent. strength are triturated with 22 grams of chromic fluoride to form a homogeneous powder.

35 14. 25.5 grams of this mixture are diazotized in the usual manner, neutralized by means of sodium acetate and made up to one liter. A diazo-solution is obtained which contains per liter 0.55 gram of chromic fluoride and the quantity of diazo-compound corresponding with 1.4 grams of 1-amino-2-methyl-4-chlorobenzene.

40 Cotton yarn is developed in this bath in the usual manner. The yarn has previously been grounded with a solution prepared as described in Example 11 from 4 grams of 1-(2',3'-hydroxy-

naphthoylamino)-2-methyl-4-chlorobenzene per liter.

After the usual after-treatment there is obtained a clear bluish red tint.

5 15. Cotton yarn is impregnated at 30° C. in the vat with a solution containing per liter—

1 - (2',3' - hydroxynaphthoylamino) - 2,4 - di-methoxy-5-chlorobenzene grams 3

Caustic soda solution of 34° Bé cc 6

10 Formaldehyde of 33 per cent. strength cc 3

Turkey red oil cc 10

squeezed and developed in the vat in a diazo-solution, neutralized by means of sodium acetate and containing per liter the amount of diazo-compound corresponding with 2.35 grams of 1-amino-2 - methoxybenzene-5 - sulfonyl-diethylamine and 3.2 grams of chromic acetate, the yarn is then after-treated in the usual manner.

20 A clear bluish red tint is thus obtained.

16. Cotton piece goods are impregnated on a foulard with a solution prepared in the usual manner from—

25 1 - (2',3' - hydroxynaphthoylamino) - naphthalene grams 10

Caustic soda solution of 34° Bé cc 20

Turkey red oil cc 15

then dried and developed on a foulard in a diazo-solution neutralized by means of sodium bicarbonate and containing per liter the amount of diazo-compound corresponding with 5.5 grams of 4,4'-diamino-3,3'-dimethoxy-diphenyl and 14 grams of chromic acetate. The dyeing is thoroughly rinsed, while cold, and soaped at boiling temperature for a short time.

An even reddish blue tint is obtained.

17. A mixed tissue, consisting of viscose artificial silk and cotton, is padded with a solution containing per liter—

2.3-hydroxynaphthoyl-aminobenzene grams 12

Caustic soda solution of 34° Bé cc 18

Turkey red oil cc 20

45 and then dried. The material thus treated is then developed on a foulard in a solution prepared by diazotizing 12.5 grams of 1-amino-4-benzoylamino-2,5-di-methoxybenzene, neutralizing by means of sodium bicarbonate, adding 20 grams of chromic acetate and making up to 1 liter. If desired, this solution is standardized by adding 20 per cent. of water.

55 At the end of the operation the material is rinsed and soaped at boiling temperature.

A uniform reddish navy-blue tint is thus obtained.

18. Bleached and desized linen-piece goods are padded, while hot, with a solution containing per liter—

2.3-hydroxynaphthoyl-aminobenzene grams 10

Caustic soda solution of 24° Bé cc 15

Turkey red oil cc 20

65 and then dried.

The material thus treated is then developed on a foulard with a solution prepared by diazotizing 11 grams of 1-amino-4-benzoylamino-2,5-diethoxybenzene, neutralizing by means of sodium bicarbonate, adding 15 grams of chromic acetate and making up to 1 liter. Finally the material is rinsed and soaped at boiling temperature.

75 An indigo blue piece dyeing is obtained.

By using instead of 2,3-hydroxynaphthoylaminobenzene the 1-(2',3'-hydroxynaphthoylamino)-2-methyl-4-chlorobenzene, there is also obtained an even indigo blue piece dyeing having a good through-dyeing effect.

A blue-green dyeing is obtained by using 1-(2'-hydroxyanthracene-3'- carbonylamino) - 2-methylbenzene as coupling component.

19. 44.9 grams of press cake of 78 per cent. strength of 4'-methoxy-diphenylamine-4-diazonium chloride are triturated to a homogeneous powder with 9.4 grams of anhydrous sodium sulfate and 45.7 grams of chromic acetate. 100 grams of a diazo-salt are obtained which is very stable to storage and contains 35 per cent. of 4'-methoxy-diphenylamine-4 - diazonium chloride.

Bleached cotton material is padded on a foulard in a solution containing per liter—

2.3-hydroxynaphthoyl-aminobenzene grams 15

Caustic soda solution of 34° Bé cc 22.5

Turkey red oil cc 20

and then dried.

The material thus treated is developed by passing it on a foulard through a solution containing per liter 43.7 grams of the above described dye-salt from 4-amino-4'-methoxy-diphenylamine, squeezed, rinsed after a passage in the air for 30 seconds, and soaped at boiling temperature.

A very uniform blue tint is obtained.

The same good result is attained if instead of the cotton material there is used a material made from artificial silk staple fibers.

20. Bleached cotton fabric is padded on a foulard in a solution containing per liter—

2.3-hydroxynaphthoyl-aminobenzene grams 15

Caustic soda solution of 34° Bé cc 22.5

Turkey red oil cc 20

and then dried.

The fabric thus treated is printed (a) with a printing paste containing per kilo—

Grams

Lactic acid of 50 per cent. strength 200

Water 300

Neutral starch-tragacanth-thickening 500

and (b) with a printing paste containing per kilo—

Acid 1,5-naphthalenedisulfonate, neutralized by means of sodium carbonate, of diazo-

tized 1-amino-2-methyl - 4 - chlorobenzene

grams 32

Crystallized aluminum sulfate do 80

60

After drying the fabric is passed through a solution of the following composition:

Diazonium chloride of 4-amino-diphenyl-

amine grams 13.47

Crystallized chromic acetate do 20

per liter of water of 25° C., then squeezed and after exposing it to air for 30 seconds passed through a bath containing per liter of water of 70° C. 10 cc. of a sodium bisulfite solution of 38° Bé, rinsed and soaped at boiling temperature.

In this way, white and red effects on navy-blue ground are obtained.

21. A mixed fabric consisting of cotton and

artificial silk staple fiber is padded in a solution containing per liter—  
 2.3-hydroxynaphthoylaminobenzene—grams 12  
 Turkey red oil—cc. 15  
 5 Caustic soda solution of 34° Bé.—cc. 18  
 and then dried.

The fabric thus treated is printed with the following printing paste:

|                                                           | Grams |
|-----------------------------------------------------------|-------|
| 10 Diazonium chloride of 4-amino-4'-methoxy-diphenylamine | 9     |
| Crystallized chromic acetate                              | 24    |
| Neutral starch-tragacanth-thickening                      | 500   |
| 15 Water                                                  | 467   |
|                                                           | 1000  |

After drying, the fabric is passed through a hot sodium carbonate solution (2 grams of calcined sodium carbonate per liter), then rinsed and soaped.

A deep fast blue print of very good evenness is obtained.

22. Cotton piece goods are impregnated on a foulard in a solution containing per liter 10 grams of 1-(2'-hydroxycarbazole-3'-carbonylamino)-4-chlorobenzene, 20 cc. of caustic soda solution of 34° Bé. and 15 cc. of Turkey red oil and dried. The dyeing is then developed on a foulard in a diazo solution, neutralized with sodium bicarbonate and containing the amount of diazo-compound corresponding with 5 grams of 1-amino-2-methoxy-5-chlorobenzene per liter and 14 grams of chromic acetate per liter. A uniform tobacco brown dyeing is obtained.

23. Cotton piece goods are impregnated on a foulard in a solution containing per liter 10 grams of 1-(3'-hydroxydiphenylene-oxide-2'-carbonylamino)-2.5-dimethoxybenzene, 20 cc. of caustic soda solution of 34° Bé. and 15 cc. of Turkey red oil and dried. The dyeing is then developed on a foulard in a diazo solution, neutralized with sodium bicarbonate and containing the amount of diazo-compound corresponding with 7 grams of 1-amino-2-methoxybenzene-5-sulfonic acid-diethylamide per liter and 14 grams of chromic acetate per liter. A uniform dark brown dyeing is obtained.

24. Cotton yarn is impregnated in the vat at 30° C. in a solution containing per liter 1.5 grams of 1-(2'-hydroxy-7,8-benzocarbazole-3'-carbonylamino)-4-methoxybenzene, 3 cc. of alcohol, 6.5 cc. of caustic soda solution of 34° Bé., 10 cc. of Turkey red oil and 1.5 cc. of formaldehyde of 33 per cent. strength, for 30 to 40 minutes, the proportion of the goods to the liquor being 1:20; the yarn is squeezed and developed in the vat for 20 minutes, the proportion of the goods to the liquor being 1:20, in a diazo solution which has been neutralized with prepared chalk and mixed with 1 gram of chromic acetate and contains the amount of diazo compound corresponding with 1.65 grams of 1-amino-2-methoxy-4-nitrobenzene per liter. After thoroughly rinsing the dyeing is soaked at boiling temperature for 30 minutes. A deep greenish black tint is thus obtained.

I claim:

1. Process of producing water-insoluble azo dyestuffs on the fiber according to the ice-color

method which comprises developing the vegetable fiber impregnated with a coupling component adapted for the production of ice-colors in a solution of a diazonium salt containing a water-soluble chromic salt as alkali binding agent.

2. Process of producing water-insoluble azo dyestuffs on the fiber according to the ice-color method which comprises developing the vegetable fiber impregnated with a 2,3-hydroxynaphthoic acid arylamide in a solution of a diazonium salt containing a water-soluble chromic salt as alkali binding agent.

3. Process of producing water-insoluble azo dyestuffs on the fiber according to the ice-color method which comprises developing the vegetable fiber impregnated with a 2,3-hydroxynaphthoic acid arylamide in a solution of a diazonium salt containing chromic acetate as alkali binding agent.

4. Process of producing a water-insoluble azo dyestuff on the fiber according to the ice-color method which comprises developing the vegetable fiber impregnated with 1-(2',3'-hydroxynaphthoylamo)-2-methyl-4-chlorobenzene in a solution of diazotized 1-amino-4-benzoylamino-2,5-diethoxybenzene containing chromic acetate as alkali binding agent.

5. Process of producing water-insoluble azo dyestuffs on the fiber according to the ice-color method which comprises developing the vegetable fiber impregnated with a coupling component adapted for the production of ice-colors in a solution of a diazo-preparation comprising a diazonium salt in solid form and a water-soluble chromic salt.

6. Process of producing water-insoluble azo dyestuffs on the fiber according to the ice-color method which comprises developing the vegetable fiber impregnated with a 2,3-hydroxynaphthoic acid arylamide in a solution of a diazo-preparation comprising a diazonium salt in solid form and a water-soluble chromic salt.

7. Process of producing water-insoluble azo dyestuffs on the fiber according to the ice-color method which comprises developing the vegetable fiber impregnated with a 2,3-hydroxynaphthoic acid arylamide in a solution of a diazo-preparation comprising a diazonium salt in solid form and chromic acetate.

8. Process of producing a water-insoluble azo dyestuff on the fiber according to the ice-color method which comprises developing the vegetable fiber impregnated with 2,3-hydroxynaphthoylaminobenzene in a solution of a diazo-preparation comprising 4'-methoxydiphenylamine-4-diazonium chloride, chromic acetate and anhydrous sodium sulfate.

9. Preparations for dyeing and printing comprising a diazonium salt in solid form and a water-soluble chromic salt.

10. A preparation for dyeing and printing comprising the diazonium chloride from 4-amino-4'-methoxydiphenylamine and chromic acetate.

11. A preparation for dyeing and printing comprising the diazonium chloride from 4-aminodiphenylamine, chromic oxalate and anhydrous sodium sulfate.

KARL JELLINEK.